

# United States Patent [19]

Kumai et al.

[11] 3,881,933

[45] May 6, 1975

[54] **LIGHT-SENSITIVE MATERIAL  
UNDERGOING LITTLE CHANGE OF  
LATENT IMAGE FORMED THEREIN**

[75] Inventors: **Akira Kumai; Keisuke Shiba; Nobuo Yamamoto, all of Minami Ashigara, Kanagawa, Japan**

[73] Assignee: **Fuji Photo Film Co., Ltd., Minami Ashigara, Kanagawa, Japan**

[22] Filed: **Sept. 17, 1973**

[21] Appl. No.: **397,490**

**Related U.S. Application Data**

[63] Continuation of Ser. No. 254,720, May 18, 1972.

**Foreign Application Priority Data**

May 18, 1971 Japan..... 46-33429

[52] U.S. Cl..... 96/111; 96/27 R; 96/126

[51] Int. Cl. .... G03c 1/30; G03c 1/14

[58] Field of Search ..... 96/111, 126, 137, 27

[56] **References Cited**

**UNITED STATES PATENTS**

3,106,468 10/1963 Burness..... 96/111  
3,128,184 4/1964 Lowe ..... 96/111

|           |         |                        |        |
|-----------|---------|------------------------|--------|
| 3,138,461 | 6/1944  | Ryan.....              | 96/111 |
| 3,174,861 | 3/1965  | Himmelmann et al. .... | 96/111 |
| 3,305,376 | 2/1967  | Burness et al. ....    | 96/111 |
| 3,542,549 | 11/1970 | Emmi.....              | 96/111 |
| 3,647,466 | 3/1972  | Bruengger et al. ....  | 96/137 |
| 3,671,260 | 6/1972  | Oftedahl et al. ....   | 96/126 |

*Primary Examiner—J. Travis Brown  
Attorney, Agent, or Firm—Rothwell, Mion, Zinn & Macpeak Sughrue*

[57] **ABSTRACT**

A gelatino-silver halide photographic emulsion containing

1. at least one of a monomethine or a trimethine cyanine dye having a cathode polarographic half wave potential ranging from 0.9 and 1.8 volt and an anode polarographic half wave potential lower than 1.3 volt and capable of forming J-aggregate, and
2. an organic compound which causes bridging to effect a hardening action and, at the same time, reacts with gelatin releasing an organic or an inorganic acid is disclosed.

**11 Claims, No Drawings**

**LIGHT-SENSITIVE MATERIAL UNDERGOING  
LITTLE CHANGE OF LATENT IMAGE FORMED  
THEREIN**

This is a continuation of application Ser. No. 254,720, filed May 18, 1972.

**BACKGROUND OF THE INVENTION**

**1. Field of the Invention**

The invention relates to a photographic light-sensitive material and, more particularly, it relates to a light-sensitive material comprising at least one light-sensitive layer which comprises a gelatino-silver-halide emulsion sensitized with a sensitizing dye.

**2. Description of the Prior Art**

Gelatino-silver-halide emulsions sensitized with dyes are used for a black and white panchromatic film or a color film, and are particularly important for color films having multi-layer type emulsion layer.

It is well known to one skilled in the art that a certain kind of dyes belonging to the cyanine dyes change the spectral sensitivity of the photographic emulsion when added to a gelatino-silver-halide emulsion. It is also publicly known that this spectral sensitization caused by the addition of a particular dye varies depending upon the type of emulsion used. In addition, it is possible that changes in various conditions in the particular photographic emulsion changes the behavior of the spectrally sensitizing agents.

Silver halide emulsions spectrally sensitized by the addition of dyes are especially of importance in a color film. Because, usually, a color film comprises three different silver halide emulsion layers, each of which records different spectral regions of blue, green and red, respectively, and, after the development, each forms a yellow, a magenta and a cyan dye image, respectively.

However, as has already been reported in *Photographic Science and Engineering*, Vol. 3, No. 3 page 134 et seq. (1969), it is well known that, when added to an emulsion certain sensitizing dyes have little effect on latent image-regression while others retard regression and even cause image-intensification.

However, especially, color roll films for camera use are often left in a camera for a fairly long period of time after exposure to light before being processed in a prescribed manner.

The best color reproduction can be obtained only when the dye images formed in each of the layers are exactly balanced with each other. Accordingly, it is quite important that the latent images formed in each layer by the exposure to light should not change during the strong period before development, or that at least they should not change in a different way from each other. That is, there is a group of sensitizing dyes which are, as is described above, excellent for the spectral sensitization of the photographic emulsion, but which are not preferred because they increase the change of the latent image with the lapse of time, the image being formed by exposure to light in the photographic emulsion to which the sensitizing dyes are added.

The inventors have now found that this change in the latent image with the lapse of time can be reduced by adding a suitable substance to a photographic emulsion layer together with these sensitizing dyes.

Therefore, a first object of the invention is to obtain a gelatino-silver-halide photographic emulsion layer which is spectrally sensitized by a sensitizing dye having an excellent spectral sensitizing action in a specific

wavelength region and, at the same time, undergoes little change of the latent image with the lapse of time, the latent image being formed therein by exposure to light.

5 Another object of the invention is to obtain a color film whose gradation and color reproduction do not change even when left for a fairly long period of time after exposure to light and before development.

Other objects of the invention will become apparent 10 by the following description and the examples.

In the case of the photographic emulsion to be treated by a processing solution, it is especially preferable that the gelatin contained therein should be durable in an aqueous solution thereof. It is especially preferred 15 that this gelatin layer should become durable in the aqueous solution at an elevated temperature as well as at an ordinary temperature since the gelatino-silver-halide photographic emulsion layer can be processed rapidly in a short time by processing it at an elevated 20 temperature. Therefore, many hardeners which are capable of making the gelatin membrane durable in an aqueous solution heated to the higher temperature are known to one skilled in the art and, in fact, they are added to a silver halide photographic emulsion layer.

25 For example, chromium alum, glyoxal, formaldehyde, 2,3-di-bromo-malealdehydic acid, the sodium salt of 2,4-di-chloro-6-hydroxy-S-triazine, etc. are well known.

However, among these hardeners, there are many 30 which are excellent in gelatin membrane-hardening action, but which deteriorate the photographic properties of the emulsion by releasing acid when reacted with gelatin molecules. For example, among the above mentioned hardeners, the sodium salt of 2,4-di-chloro-6-hydroxy-S-triazine releases hydrochloric acid, while 2,3-di-bromo-malealdehydic acid releases hydrobromic acid, and other hardeners such as 2-phenoxy-3-chloro-malealdehydic acid releases carbolic acid thus lowering the pH value of the dry emulsion membrane.

35 40 The lowering of the pH in the emulsion layer by the production of acids will cause various changes in the photographic properties and, above all, it is well known to one skilled in the art that it can cause fading of the latent image formed in the emulsion layer with the passage of time (see, for example, *Veroeffentlichungen des Wissenschaftlichen Zentral Laboratoriums der Photographicen Ableitung Agfa* Vol. 3 pages 47-52 (1933)).

45 Actually, while 2,4-dichloro-S-triazine derivatives are excellent gelatin hardeners, they have the disadvantage that the latent images formed in a gelatino-silver-halide photographic emulsion layer hardened by the addition thereof will fade with the lapse of time after exposure.

50 The tendency toward fading of latent image is increased by the use of this type of hardener, which has already been reported, for example, about [b]-type hardeners described below in *Photographische Korrespondenz* Vol. 105, pages 28-29 (1969) with data.

**SUMMARY OF THE INVENTION**

55 60 The inventors have now found that a spectrally sensitized photographic emulsion layer which undergoes extremely little change of the latent image formed therein with the lapse of time can be obtained by adding, among these hardeners, such an organic compound (a gelatin hardener) that produces an organic or an inorganic acid, to the gelatino-silver-halide emulsion layer sensitized in a specific spectral region by the use of

65

spectrally sensitizing dyes which have a latent image-intensifying action as is described herein, whereby the opposing actions of the two toward the change of the latent image with the lapse of time successfully counteract each other.

## DETAILED DESCRIPTION OF THE INVENTION

As is apparent from the description above, even when "such hardeners that have the disadvantage that, while they are excellent in gelatin-hardening action, fading, with the lapse of time, of the latent image formed in the gelatino-silver-halide emulsion layer to which these hardeners are added increases according to a conventional manner" are used, a light-sensitive layer which is excellent in gelatin-hardening action and undergoes little fading of the latent image formed therein can be obtained by the present invention. 10 15

The sensitizing dyes employed in the invention give high spectral sensitivity and, at the same time, have an effect of giving strong latensification. The monomethine or trimethine cyanine dyes used for the invention have the characteristics of forming J-aggregate and having a cathode polarographic half wave potential between  $-0.9$  and  $-1.8$  volt and an anode polarographic half wave potential lower than  $1.3$  volt. with respect to the J-aggregate, refer for example to C. E. K. Mees *The Theory of the Photographic Process Revised*; Macmillan, pp. 442 to 444, 450 to 459, 467, 475 or *ibid* the Third Edition, pp. 214, 240, 245, 254, 268. Furthermore, from the stand point of quantum theory, it is desirable that, in the state wherein the J-aggregate is formed on the surface of silver halide, the minimum vacant electron energy level should be in the vicinity of the conduction band of the silver halide, preferably, a little higher than that, and that the normal electron energy level should be higher than the valence electron band of the silver halide.

The general formulae of the sensitizing dyes used in the invention are as follows. General formula (I)



wherein  $Y_3$  represents an oxygen atom, a selenium atom, a  $=N-R_6$  group or a



group,  $R_7$  and  $R_8$  each represents a methyl group or an ethyl group,  $R_5$  and  $R_6$  each represents a lower alkyl group having, preferably 1 to about 6 carbon atoms, an allyl group or a substituted alkyl group,  $R_3$  and  $R_4$ , each represents a lower alkyl group having, preferably 1 to about 6 carbons atoms, an allyl group or a substituted alkyl group,  $Z_3$  and  $Z_4$  each represents the non-metallic atoms necessary to complete a benzene or a naphthalene nucleus,  $X_2^-$  represents an anionic group usually used for cyanine dyes,  $q$  represents an integer of 1 or 2, and, when  $q$  represents 1 an intramolecular salt is formed.

The dyes used for the invention have the characteristic of forming J-aggregate.

35 In the general formula (I), the benzene or naphthalene nucleus completed by  $Z_1$  or  $Z_2$  may be substituted with a lower alkyl group having, preferably 1 to about 6 carbon atoms, a halogen atom, an alkoxy carbonyl group, a phenyl group, an alkoxy group having preferably 1 to about 4 carbon atoms, a hydroxy group, etc. In the general formula (II), the benzene or naphthalene nucleus completed by  $Z_3$  or  $Z_4$  may be substituted by a hydrogen atom, a cyano group, an alkoxy carbonyl group, a trifluoromethyl group, an alkylsulfonyl group, an alkylsulfamoyl group, an alkylcarbamoyl group, an acetoxy group, a lower alkyl group having, preferably, 1 to about 4 carbon atoms, an alkoxy group, etc. In the general formula (I) or (II), examples of suitable lower alkyl groups represented by  $R_1$ ,  $R_2$ ,  $R_3$ ,  $R_4$ ,  $R_5$  or  $R_6$  are methyl, ethyl, propyl, butyl, etc., and examples of the substituted alkyl groups are hydroxyalkyl groups (e.g., a beta-hydroxyethyl group), acetoxyalkyl groups (e.g., beta-acetoxyethyl, gamma-acetoxypropyl groups), 55 aralkyl groups (e.g., a benzyl group), substituted alkyl groups having a sulfo or carboxy group (e.g., gamma-sulfopropyl, delta-sulfobutyl, 2-(3-sulfopropoxy)-ethyl, 2-[2-(3-sulfopropoxy)ethoxy]ethyl, beta-carboxyethyl, gamma-carboxypropyl, delta-carboxybutyl groups), 60 etc., and, for example, those described in German Pat. No. 929,080, U.S. Pat. Nos. 2,537,880 and 2,776,280, British Pat. No. 1,001,480, Japanese patent publication Nos. 4834/60, 14112/65, 23467/65, 2607/67, 15894/70, 27672/70, 27673/70 and 32740/70, and the like are used. Examples of the group A in the general formula (I) are a hydrogen atom, a methyl group, an ethyl group, a propyl group, a phenethyl group, a benzyl group, etc. Examples of  $X_1^-$  and  $X_2^-$  are a bromide 65



wherein  $Y_1$  and  $Y_2$  each represents an oxygen atom, a sulphur atom, a selenium atom or a  $-\text{CH}=\text{CH}-$  group,  $Z_1$  and  $Z_2$  each represents the non-metallic atoms necessary to complete a benzene or naphthalene nucleus,  $n$  represents an integer of 1 or 2,  $X_1^-$  represents an anionic group usually used for cyanine dyes,  $P$  represents an integer of 1 or 2, and, when  $p$  represents 1 an intramolecular salt is formed,  $R_1$  and  $R_2$ , each represents a lower alkyl group having, preferably, 1 to about 6 carbon atoms, an allyl group or a substituted alkyl group, and  $A$  represents a lower alkyl group having, preferably, 1 to about 3 carbon atoms or a substituted alkyl group. General formula (II)

ion, an iodide ion, a p-toluenesulfonate ion, a perchlorate ion, an ethylsulfate ion, a benzenesulfonate ion, etc.

Specific examples of the sensitizing dyes used in the invention are as follows, but the invention is not to be interpreted to be limited only to them.

(A)



Eox(volt) Ered(volt)

1.041 -1.036

(B)



1.131 -1.215

(C)



Eox(volt) Ered(volt)

0.535 -1.500

(D)



0.903 -1.231

(E)



0.514 -1.581

(F)



Eox(volt    Ered(volt)  
0.535       -1.500

(G)



0.519       -1.520

(H)



0.525       -1.541

(I)



(J)



0.818       -1.306



0.743 -1.401



3,881,933

11

12

(P)



0.767 -1.176

(Q)



0.535 -1.500

(R)

Eox(volt) Ered(volt)  
0.606 -1.331

(S)



0.941 -0.936

(T)



1.164 -1.127

Compound (V) is an example of a sensitizing dye and in addition a supersensitizing agent which can be used together with the sensitizing agent used in the invention. The sensitizing dye of the invention may be used either independently or in combination with other dyes or one or more of the above described dyes, as a supersensitizing agent.

That is, some of the sensitizing dyes of the invention are sensitizing dyes and in addition are also supersensitizing agents, for example

25831/70, 1999/71, and 3699/71, German OLS Nos. 1,772,956; 1,811,542; 1,929,037; 2,011,879; 2,014,896; 2,017,053; 2,030,326; and 2,031,491, etc. can also be applied thereto.

5 Among the cyanine dyes represented by the general formula (I) or (II), especially preferable dyes are those represented by one of the following general formula (III) to (VI). General formula (III):

10



15

(U)



In addition to the foregoing, supersensitizing agent the sensitizing art described in the Japanese patent publication Nos. 4932/68, 4933/68, 4936/68, 22884/68, 2530/69, 32753/69, 26470/70, 27671/70,

30

wherein Y<sub>1</sub>, Z<sub>1</sub> and Z<sub>2</sub> are the same as defined in the general formula (I), and R<sub>9</sub> and R<sub>10</sub> each represents a sulfoalkyl group, which may be the same or different.

Additional specific examples thereof are as follows.





General formula (IV):



wherein  $R_{11}$  and  $R_{12}$  each represents a sulfoalkyl group, which may be the same or different,  $W_1$ ,  $W_2$ ,  $W_3$  and  $W_4$ , each represents a chlorine atom, a bromine atom,

a trifluoromethyl group, and alkoxy carbonyl group or an alkylsulfonyl group.

For example, the following compound is illustrative.



General formula (V):



wherein  $\text{R}_1$ ,  $\text{R}_2$ ,  $\text{X}_1$  and  $p$  are the same as defined in the general formula (I).

Specific examples thereof are as follows.



General formula (VI):



wherein  $Z_1$ ,  $Z_2$ ,  $R_1$ ,  $R_2$ ,  $X_1$  and  $p$  are the same as defined in the general formula (I).

Specific examples thereof are as follows.



The aforesaid cathode polarographic half wave potential  $E_{\text{red}}$  can be strictly measured by volt-ammmetry. This is, it is measured in an acetonitrile solution ( $1 \times 10^{-4}$  mol— $1 \times 10^{-6}$  mol) at  $25^\circ\text{C}$  with the use of a dropping mercury electrode using saturated calomel electrode as a reference electrode, and using tetra-n-propylammonium perchlorate as a supporting electrolyte. The anode polarographic half wave potential  $E_{\text{ox}}$  can be measured in the same manner as in the  $E_{\text{red}}$  value with the use of a rotating platinum electrode using sodium perchlorate as a supporting electrolyte. A more detailed procedure is described in the German O.L.S. No. 2,010,762.

The sensitizing dyes employed in the invention are used, preferably, in an amount of from  $1 \times 10^{-6}$  to  $1 \times 10^{-3}$  mol per 1 mol of silver halide. The amount of the dye can be varied depending on the property of the emulsion and the dye employed. The sensitizing dyes are added in any conventional manner, for example, by dissolving them in water, methanol, ethanol, pyridine, methyl cellosolve, acetone, etc. Other procedures described in Japanese Patent Application No. 8231/70, Japanese patent publication No. 23389/69, 27555/69, and 22948/69, U.S. Pat. No. 3,485,634; 3,342,605; and 2,912,343, German O.L.S. No. 1,947,935, etc. may be used.

The gelatin hardeners used according to the invention are those which react with gelatin and cause bridging to effect a hardening action and, at the same time, produce an organic or an inorganic acid as a by-product. Examples of those which release hydrohalic acids are 2,3-dihalogenomalealdehydic acids (U.S. Pat. No. 2,080,019), 2,4-dichloro-S-triazines (U.S. Pat. No. 3,325,287), chloropyrimidine derivatives (British Pat. No. 1,193,290), polymers having a chlorotriazine ring as a side chain (U.S. Pat. No. 3,362,827, German O.L.S. No. 1,921,363), dichlorophosphoamide derivatives (British Pat. No. 974,723, and 1,004,658, U.S. Pat. No. 3,125,449), halomethyl derivatives (British Pat. No. 990,275), and phosphonitrilechloride derivatives (U.S. Pat. No. 3,186,848). Examples of those which release phenol derivatives are 2-phenoxy-3-halogeno-malealdehydic acid derivatives (British Pat. No. 1,192,775, U.S. Pat. No. 3,579,374), etc. Especially preferred hardeners are organic compounds which release hydrochloric acid, hydrobromic acid, carbolic acid, or carboxylic acid derivatives. In practice, these gelatin hardeners are dissolved in a solvent which is miscible with water and does not affect the photographic emulsion, such as water, methanol, dimethyl-

formamide, etc. and added at an any stage before coating them onto the emulsion. Suitable hardening effects can be brought about by adding them in an amount of, preferably, from 1 to 100 g, and in an optimum range, from 5 to 60 g, per 1 kg based on the dry weight of the gelatin contained in a coating composition which contains gelatin.

Specific examples of the above described hardeners are as follows.

(a)  $\text{Cl}-\overset{\text{Cl}}{\underset{\text{H}}{\text{C}}}-\text{COOH}$   
 $\text{Cl}-\overset{\text{Cl}}{\underset{\text{H}}{\text{C}}}-\text{CHO}$



(f) Copolymer of 80 mol % of the compound represented by the following formula;

$$\text{CH}_2=\overset{\text{CH}_3}{\underset{\text{CH}_3}{\text{C}}}-\text{CO}-\text{O}-\text{CH}_2-\text{NH}-\text{C}_6\text{H}_4-\text{Cl}$$

and 20 mol % of acrylic acid.



The gelatino-silver-halide photographic emulsions used according to the invention are high speed emulsions, especially, a silver bromoiodide emulsion. However, the present invention is applicable to other silver halide emulsions such as silver chlorobromide, pure silver bromide, etc. A high speed silver bromoiodide emulsion usually contains less than 10 mol percent of silver iodide, and is usually chemically sensitized with a sulfur sensitizing agent and/or a gold sensitizing agent to such an extent that optimum sensitivity is obtained, and is further spectrally sensitized with the aforesaid spectrally sensitizing agents. As sulfur sensitizing agents, sodium thiosulfate, triethylthiourea, allylisothiourea and, as gold sensitizers,  $\text{HAuCl}_4 \cdot 4\text{H}_2\text{O}$ ,  $\text{AuSCN}$ , etc. may be used in a conventionally known manner. In addition, various palladium compounds such as palladium chloride can also be used in combination.

As anti-fogging agents, benzotriazole, nitrobenzimidazole, 5-nitroindazole, 1-phenyl-5-mercaptotetrazole, 4-hydroxy-6-methyl-1,3,3a,7-tetrazaindene, etc. are used.

As coating agents, anionic and non-ionic agents such as saponin, sodium dodecylbenzenesulfonate, sucrose monolaurate, polyethyleneglycol nonylphenylether, etc. can be added in a suitable amount.

The invention is applicable for usual black and white films or multi-layer color sensitive materials containing no color coupler and, in addition, it is also applicable to a superposed color sensitive material wherein an emulsion spectrally red-sensitized with spectrally sensitizing agents and containing a cyan coupler, an emulsion spectrally green-sensitized with spectrally sensitizing agents and containing a magenta coupler, a yellow filter layer which can be bleached, and a blue sensitive emulsion containing a yellow coupler, are coated on a support in turn. Each layer is often coated in the order described above. However, this order can be altered depending upon the purpose of use. Furthermore, auxiliary layers such as a filter layer, an intermediate layer, an anti-halation layer, a protective layer, etc. may be additionally provided. The emulsions are coated, for example, on paper, polymer laminated paper, glass, cellulose triacetate, or films of synthetic filmforming resin such as polyesters, polyamides, polystyrenes, etc. Of the above supports, cellulose triacetate and polyesters are prefered. A suitable coating amount of the emulsion is prefered to be within a range of from about 20 to about 200 mg of silver per  $100\text{cm}^2$  or a thickness of from about 5 to 30  $\mu$  of emulsion after drying.

The invention will now be explained in greater detail by reference to the following examples which are for the purposes of illustration.

#### EXAMPLE 1

500 g portions of a high speed gelatino-silver- 60 bromoiodide negative emulsion (5.5 mol percent in sil-

ver iodide content) containing 0.32 mol of silver halide per 1 kg were weighted out, and heated to 40°C to dissolve, the emulsion being previously chemically sensitized with sodium thiosulfate and chloroauric acid in a conventional way to such an extent that suitable sensitivity can be obtained. The spectrally sensitizing dyes given in the table I were added to the emulsions with stirring and, after stirring for an additional 15 minutes, were allowed to stand. To these were added 20 cc portions of a 1 percent aqueous solution of 4-hydroxy-6-methyl-1,3,3a,7-tetrazaindene, then, the hardeners described in Table I were added thereto and, in addition, 5 cc portions of a 4 percent saponin aqueous solution were added. Thereafter, the emulsions were coated on a cellulose triacetate film base previously undercoated, then dried.

On the other hand, in the measurement of the melting point of the emulsion membrane, the melting point was determined by raising the temperature of water wherein each sample having been coated three days before was dipped, until the emulsion membrane melted or peeled from the film base. The temperature at which these phenomena occurred was regarded as the melting point.

Then, four strips were cut from each of the emulsion-coated samples for testing, and two of them (1) and (2) were exposed to a tungsten light source (2854°K) through a blue filter (a BPN45 filter made by the Fuji Photo Film Co., Ltd.) and a yellow filter (an SC-50 filter made by the Fuji Photo Film Co., Ltd.), respectively, and both through a neutral wedge. After leaving for 5 days at 50°C under a 70 percent relative humidity, these were developed for 4 minutes at 20°C with the use of a developer having the following composition.

Immediately before this development, the other two strips (3) and (4) which had been stored in a room at a temperature of -20°C for these 4 days were exposed in the same manner as described above, and developed at the same time as (1) and (2), and additionally, fixed, washed, dried to obtain negative images. The H and D curves were drawn in a conventional manner using an optical densitometer, and the sensitivity at the point of an optical density of +0.2 in fogging was calculated. The sensitivity is given in the table as the ratio of the sensitivity of (1) or (2) to that of (3) or (4). These values can be regarded as a "measure of the rate of change of the latent image" in the case in which the samples were left for 4 days at 50°C under a 65 percent relative humidity. This storage condition is known to correspond to the case of being left for about 3 months in a usual room condition.

| Composition of the Developer: |            |      |
|-------------------------------|------------|------|
| Metol                         | 0.3        | g    |
| Potassium Pyrosulfite         | 1.4        | g    |
| Anhydrous Sodium Sulfite      | 38         | g    |
| Hydroquinone                  | 6          | g    |
| Sodium carbonate monohydrate  | 22.5       | g    |
| Citric Acid                   | 0.7        | g    |
| Water                         | to make up | 1000 |
|                               |            | cc   |

Table 1

| Test No. | Sensitizing Dye         | Hardener | Changing Ratio of Latent Image (%) (50°C, 65% RH, for 4 days) | M.P. of Sample                                     |
|----------|-------------------------|----------|---------------------------------------------------------------|----------------------------------------------------|
|          | (mol concentration)     | cc       | g/Kg gelatin                                                  | (1)/(3) (blue filter) (2)/(4) (yellow filter) (°C) |
| 1        | A (1×10 <sup>-3</sup> ) | 10       | —                                                             | 117 117 32                                         |
| 2        |                         | 20       | —                                                             | 142 142 32                                         |
| 3        |                         | 40       | —                                                             | 160 160 32                                         |
| 4        |                         | —        | a 3                                                           | 80 80 54                                           |
| 5        |                         | —        | a 5                                                           | 72 72 72                                           |
| 6        |                         | 10       | a 5                                                           | 96 96 72                                           |
| 7        |                         | 20       | a 5                                                           | 102 106 74                                         |
| 8        |                         | 40       | a 5                                                           | 120 120 72                                         |
| 9        | B (1×10 <sup>-3</sup> ) | 10       | —                                                             | 117 117 32                                         |
| 10       |                         | 20       | —                                                             | 117 117 32                                         |
| 11       |                         | 40       | —                                                             | 158 160 32                                         |
| 12       |                         | —        | b 15                                                          | 90 90 46                                           |
| 13       |                         | —        | b 30                                                          | 70 70 70                                           |
| 14       |                         | 20       | b 30                                                          | 98 98 72                                           |
| 15       |                         | 40       | b 30                                                          | 108 108 72                                         |
| 16       | C (1×10 <sup>-3</sup> ) | 20       | —                                                             | 142 160 32                                         |
| 17       |                         | 40       | —                                                             | 160 160 32                                         |
| 18       |                         | —        | a 5                                                           | 72 72 72                                           |
| 19       |                         | —        | b 15                                                          | 90 90 45                                           |
| 20       |                         | 40       | a 5                                                           | 100 102 70                                         |
| 21       |                         | 40       | b 15                                                          | 110 110 46                                         |
| 22       | D (1×10 <sup>-3</sup> ) | 20       | —                                                             | 132 132 32                                         |
| 23       |                         | 40       | —                                                             | 142 142 32                                         |
| 24       |                         | 80       | —                                                             | 150 150 32                                         |
| 25       | D (1×10 <sup>-3</sup> ) | 40       | —                                                             | 200 200 33                                         |
| 26       | H (5×10 <sup>-4</sup> ) | 20       | —                                                             |                                                    |
| 27       | D (1×10 <sup>-3</sup> ) | 40       | b 30                                                          | 120 120 70                                         |
| 28       | H (5×10 <sup>-4</sup> ) | 20       | —                                                             |                                                    |
| 29       | E (5×10 <sup>-4</sup> ) | 20       | —                                                             |                                                    |
| 30       |                         | 40       | c 20                                                          | 96 96 40                                           |
| 31       |                         | —        | c 40                                                          | 78 78 95                                           |
| 32       |                         | 40       | c 20                                                          | 106 106 40                                         |
| 33       |                         | 40       | c 40                                                          | 110 110 95                                         |
| 34       | F (5×10 <sup>-4</sup> ) | 20       | —                                                             |                                                    |
| 35       | F (5×10 <sup>-4</sup> ) | 40       | —                                                             | 136 160 31                                         |
| 36       | C (1×10 <sup>-3</sup> ) | 20       | —                                                             | 160 160 32                                         |
| 37       | F (5×10 <sup>-4</sup> ) | 20       | —                                                             | 200 230 32                                         |
| 38       | C (1×10 <sup>-3</sup> ) | 20       | c 40                                                          | 136 136 90                                         |
| 39       | G (5×10 <sup>-4</sup> ) | 20       | —                                                             |                                                    |
| 40       |                         | 40       | d 20                                                          | 136 140 >100                                       |
| 41       |                         | —        | d 20                                                          | 92 92 >100                                         |
| 42       | G (5×10 <sup>-4</sup> ) | 40       | d 20                                                          | 100 100 >100                                       |
| 43       | H (5×10 <sup>-4</sup> ) | 20       | —                                                             | 106 106 >100                                       |
| 44       |                         | 40       | d 20                                                          | 136 142 >100                                       |
| 45       |                         | 40       | a 10                                                          | 160 160 32                                         |
| 46       |                         | 40       | b 30                                                          | 108 108 90                                         |
| 47       |                         | 40       | d 20                                                          | 116 112 74                                         |
| 48       | I (1×10 <sup>-3</sup> ) | 20       | —                                                             | 120 118 >100                                       |
| 49       |                         | 40       | —                                                             | 117 117 32                                         |
| 50       |                         | —        | f 10                                                          | 142 142 >100                                       |
| 51       |                         | 20       | f 10                                                          | 96 96 >100                                         |
| 52       | I (1×10 <sup>-3</sup> ) | 40       | f 10                                                          | 102 102 >100                                       |
| 53       |                         | 20       | —                                                             | 108 108 >100                                       |
| 54       |                         | 40       | a 8                                                           | 142 142 >100                                       |
| 55       |                         | 40       | a 8                                                           | 160 160 86                                         |
| 56       | J (1×10 <sup>-3</sup> ) | 40       | —                                                             |                                                    |
| 57       |                         | 80       | —                                                             | 132 142 32                                         |
| 58       |                         | —        | g 15                                                          | 142 142 32                                         |
| 59       |                         | 40       | g 15                                                          | 90 90 60                                           |
| 60       |                         | 80       | g 15                                                          | 110 116 62                                         |
| 61       | L (5×10 <sup>-4</sup> ) | 10       | —                                                             | 116 120 60                                         |
| 62       |                         | 20       | —                                                             | 117 117 32                                         |
| 63       | L (5×10 <sup>-4</sup> ) | 20       | —                                                             | 132 132 32                                         |
| 64       | A (1×10 <sup>-3</sup> ) | 20       | —                                                             | 160 178 32                                         |
| 65       | L (5×10 <sup>-4</sup> ) | 20       | g 15                                                          | 116 120 62                                         |
| 66       | A (1×10 <sup>-3</sup> ) | 20       | g 15                                                          | 85 85 62                                           |
| 67       | M (1×10 <sup>-3</sup> ) | 10       | —                                                             | 126 126 32                                         |
|          |                         | 20       | —                                                             | 126 142 31                                         |
|          |                         | 10       | e 40                                                          | 110 110 90                                         |

| Test No. | Sensitizing Dye                                    | Hardener |   | Changing Ratio of Latent Image (%) (50°C, 65% RH, for 4 days) |     | M.P. of Sample |
|----------|----------------------------------------------------|----------|---|---------------------------------------------------------------|-----|----------------|
| 68       |                                                    | 20       | e | 40                                                            | 112 | 112            |
| 69       | O (1×10 <sup>-3</sup> )                            | 20       |   | —                                                             | 136 | 112            |
| 70       |                                                    | 40       |   | —                                                             | 150 | 32             |
| 71       |                                                    | 40       | b | 15                                                            | 136 | 32             |
| 72       |                                                    | 40       | b | 30                                                            | 120 | 45             |
| 73       |                                                    | 40       | b | 45                                                            | 112 | 70             |
|          |                                                    |          |   |                                                               |     | >100           |
| 74       | U (5×10 <sup>-4</sup> )                            | 10       |   | —                                                             | 100 | 32             |
| 75       |                                                    | 20       |   | —                                                             | 110 | 31             |
| 76       |                                                    | 40       |   | —                                                             | 100 | 32             |
| 77       | U (5×10 <sup>-4</sup> )<br>M (1×10 <sup>-3</sup> ) | 10       |   | —                                                             | 152 | 32             |
| 78       | U (5×10 <sup>-4</sup> )<br>M (1×10 <sup>-3</sup> ) | 10       | h | 30                                                            | 126 | 130            |
|          |                                                    | 20       |   |                                                               |     | >100           |
| 79       | P (1×10 <sup>-3</sup> )                            | 20       |   | —                                                             | 132 | 31             |
| 80       |                                                    | 40       |   | —                                                             | 142 | 32             |
| 81       | P (1×10 <sup>-3</sup> )<br>L (5×10 <sup>-4</sup> ) | 20       |   | —                                                             | 160 | 31             |
| 82       | P (1×10 <sup>-3</sup> )<br>L (5×10 <sup>-4</sup> ) | 20       | i | 5                                                             | 130 | 72             |
|          |                                                    | 10       |   |                                                               |     |                |
| 83       | N (1×10 <sup>-3</sup> )                            | 20       |   | —                                                             | 150 | 32             |
| 84       |                                                    | 40       |   | —                                                             | 145 | 32             |
| 85       |                                                    | —        | j | 60                                                            | 86  | >100           |
| 86       |                                                    | 20       | j | 60                                                            | 110 | 86             |
|          |                                                    |          |   |                                                               |     | >100           |
| 87       |                                                    | 40       | j | 60                                                            | 116 | 116            |

No. 6, 7, 8, 14, 15, 20, 21, 26, 31, 32, 36, 40, 41, 44, 30 45, 46, 50, 51, 54, 55, 59, 60, 64, 67, 68, 71, 72, 73, 78, 82, 86 and 87 are combinations of the invention. The other test Nos. are given for comparison.

## EXAMPLE 2

35

To 1,000 parts of a coarse grained high speed silver bromoiodide photographic emulsion containing 16 g of gelatin and 6.0 g of silver bromoiodide per 100 g of the emulsion (silver iodide content being 6.0 mol percent based on the total silver halide) were added the specifically sensitizing dyes given in Table 2, 20 parts of a 1 percent aqueous solution of 4-hydroxy-6-methyl-1,3,3a,7-tetrazaindene as an anti-fogging agent 150 parts of a 5 percent alkaline solution of the cyan color coupler (T) of the following formula, hardeners given in Table 2, and, as a coating agent, 40 parts of a 1 percent aqueous solution of sodium dodecylbenzenesulfonate, in order, at 40°C with sufficient stirring, then coated on a cellulose triacetate film base previously undercoated in a conventional manner, and dried (3.3 microns in dry film thickness).

midity. The other control film strip was stored in a refrigerator at -20°C during this period, then, exposed in the same manner as described above and immediately developed according to the processing as follows together with the foregoing strips.

35

1. Color Development (at 20°C, for 8 minutes)  
Diethyl-p-phenylenediamine Sulfate 2.75 g  
Hydroxylamine Sulfate 1.2 g  
Anhydrous Sodium Sulfite 2 g  
Potassium Bromide 2 g  
Water to make up 1000 cc
2. Hardening (at 20°C, for 8 minutes)  
Anhydrous Sodium Sulfite 100 g  
Water to make up 1000 cc
3. First Fixing (at 20°C, for 5 minutes)  
Sodium Thiosulfate 150 g  
Water to make up 1000 cc
4. Washing (for 5 minutes)
5. Bleaching (at 20°C, for 5 minutes)  
Red prussiate 100 g  
Water to make up 1000 cc
6. Washing (at 20°C, for 5 minutes)
7. Second Fixing (at 20°C, for 5 minutes)  
Conducted in the same manner as the first fixing.
8. Washing (for 20 minutes)



Two film strips were cut from each of the resulting emulsion-coated substances. One of the strips was im- 65 agewise exposed to light through a yellow filter for 1/100 second using a neutral grey wedge, then kept for 1 week in a room at 50°C under 70 percent relative hu-

All of the resulting cyan dye images formed on the strips were subjected to sensitometry through a red filter using an optical densitometer. The sensitivity was measured at a fogging point of +0.2, and the relative sensitivity (%) of the sensitivity of the strip incubated

after exposure to that of the control strip was regarded as the index of the change of the latent image with the lapse of time after exposure.

The melting points of the emulsion membranes were measured in the same manner as described in Example 1.

optimum sensitivity can be obtained, then, coated on a cellulose triacetate film base having been previously undercoated in a conventional way, dried (3.5 microns in dry film thickness).

Two film strips were cut from each of the resulting seven emulsion-coated samples, and each of the two

Table 2

| Test No. | Spectrally Sensitizing Dye<br>(mol concentration) | Hardener<br>cc | Changing Ratio of Latent Image with the Lapse of Time (%)<br>(2)/(4) (yellow filter) | M.P. of Sample (°C) |
|----------|---------------------------------------------------|----------------|--------------------------------------------------------------------------------------|---------------------|
| 88       | —                                                 | —              | 92                                                                                   | 31                  |
| 89       | —                                                 | b              | 88                                                                                   | 42                  |
| 90       | —                                                 | b              | 70                                                                                   | 66                  |
| 91       | P (1×10 <sup>-3</sup> )                           | 40             | 140                                                                                  | 32                  |
| 92       | L (1×10 <sup>-3</sup> )                           | 20             | 156                                                                                  | 32                  |
|          | M                                                 | 20             |                                                                                      |                     |
| 93       | P (1×10 <sup>-3</sup> )                           | 40             | 120                                                                                  | 40                  |
| 94       | P (1×10 <sup>-3</sup> )                           | 40             | 108                                                                                  | 68                  |
| 95       | L (1×10 <sup>-3</sup> )                           | 20             | 126                                                                                  | 43                  |
|          | M                                                 | 20             |                                                                                      |                     |
| 96       | L (1×10 <sup>-3</sup> )                           | 20             | 112                                                                                  | 70                  |
|          | M                                                 | 20             |                                                                                      |                     |

In Table 2, No. 93, 94, 95, and 96 are the combinations of the invention. The other test Nos. are given for comparison.

## EXAMPLE 3

8 g of a magenta color coupler 1-(2',4',6'-trichlorophenyl)-3-3''-(2'',4''-di-tertiary-amyl-phenoxyacetamide)benzamide -5-pyrazolone was weighed out, and dissolved in a mixture of 25 cc of ethyl acetate and 4 cc of di-n-butyl phthalate at the reflux temperature of ethyl acetate. The resulting mixture was poured into a mixture of 65cc of a 10 percent gelatin aqueous solution and a 5 percent aqueous solution of sodium triisopropylnaphthalenesulfonate at 50°C in about 1 minute with sufficient stirring, then passed through a colloid mill 5 times. Thereafter, the mill was rinsed with 25 cc of water, and the resulting dispersion 40 was solidified on a cooling plate cooled to 5°C, cut into strips, air-dried at 78°C under a 50 percent relative humidity. The total dry dispersion weighed 18.5 g and, when this was re-dispersed in gelatin, the grain diameter of the dispersed grains was larger than 0.5 micron 45 and no crystal separation was observed.

Methanol solutions of the sensitizing dyes given in Table 3, 5 parts of a 1 percent aqueous solution of 4-hydroxy-6-methyl-1,3,3a,7-tetrazaindene as a fogging agent, 5 parts of the above described magenta color 55 coupler dispersion, an aqueous solution of the hardeners given in Table 3, and 3 parts of 1 percent aqueous solution of sodium dodecylbenzenesulfonate as a coating agent were added in order with sufficient stirring per 100 parts of the high speed gelatino-silver-halide negative emulsion which contained 60 g of gelatin and 60 g of silver bromoiodide (5 mol percent in silver iodide content) per 1 kg and was chemically sensitized in a conventionally known manner to such an extent that

30 film strips was exposed to a 5400°K light through a neutral grey wedge for 1/100 second, then kept in a room at 50°C under a 70 percent relative humidity for 1 week. The other control film strip was stored in a refrigerator at -20°C during this period, then, exposed in the same way as described above, and immediately developed together with the aforesaid strips at 20°C for 12 minutes using the following developer.

|                                                                  |                                                                                                              |
|------------------------------------------------------------------|--------------------------------------------------------------------------------------------------------------|
| 2-Amino-5-diethylaminotoluene Hydrochloride                      | 2 . g                                                                                                        |
| Anhydrous Sodium Sulfite                                         | 2 g                                                                                                          |
| Anhydrous Sodium Carbonate                                       | 20 g                                                                                                         |
| Potassium Bromide                                                | 2 g                                                                                                          |
| Benzyl Alcohol                                                   | 2 g                                                                                                          |
| Water                                                            | 1.0 l<br>to make up                                                                                          |
| Successively, the following processing was conducted<br>at 20°C. |                                                                                                              |
| Rinsing                                                          | 15 sec.                                                                                                      |
| Hardening and Fixing                                             | 2 min.                                                                                                       |
| Washing                                                          | 3 min.                                                                                                       |
| Bleaching                                                        | for 2 minutes using a solution<br>containing 50 g of red prussiate and<br>20 g of potassium bromide per 1 l. |
| Rinsing                                                          | 15 sec.                                                                                                      |
| Fixing                                                           | 2 min.                                                                                                       |
| Washing                                                          | 5 min.                                                                                                       |
| Drying                                                           |                                                                                                              |

60 All of the resulting magenta dye images formed on the strips were subjected to sensitometry through a green filter using an optical densitometer. The sensitivity is given as a relative sensitivity of the sample incubated at 50°C under a 70 percent relative humidity to that of the control sample.

The melting points of the samples were measured in water in a conventional way as is employed by one skilled in the art of photographic industry after a 1 week period between the coating and drying of the samples.

Table 3

| Test No. | Spectrally Sensitizing Dye | Hardener | Changing Ratio of Latent Image with the Lapse of Time (%) (2)/(4) (yellow filter) | M.P. of Sample (°C) |
|----------|----------------------------|----------|-----------------------------------------------------------------------------------|---------------------|
|          | (mol concentration)        | cc       | g/Kg gelatin                                                                      |                     |
| 97       | C ( $1 \times 10^{-3}$ )   | 40       | —                                                                                 | 172                 |
| 98       | —                          | —        | b 20                                                                              | 80                  |
| 99       | —                          | —        | e 10                                                                              | 85                  |
| 100      | C ( $1 \times 10^{-3}$ )   | 40       | b 20                                                                              | 110                 |
| 101      | C ( $1 \times 10^{-3}$ )   | 40       | e 10                                                                              | 106                 |
| 102      | D ( $1 \times 10^{-3}$ )   | 40       | —                                                                                 | 142                 |
|          | F ( $5 \times 10^{-4}$ )   | 20       |                                                                                   |                     |
| 103      | D ( $1 \times 10^{-3}$ )   | 40       | b 20                                                                              | 100                 |
|          | E ( $5 \times 10^{-4}$ )   | 20       |                                                                                   | 60                  |

As is obvious from the results contained in Tables 1 to 3, in the combination of the sensitizing dye and the hardener in the invention, the changing rate of the latent image with the lapse of time is extremely near the ideal of 100 percent or no change. Therefore the object of the invention has effectively completed.

On the other hand, in the samples prepared for comparison, it can be seen that the changing rate deviates relatively greatly from the ideal 100 percent.

While the invention has been described in detail and in terms of various embodiments thereof, it will be apparent to one skilled in the art that various changes and

compound which causes bridging to effect a hardening action by reaction with gelatin and, at the same time, reacts with gelatin releasing an organic or an inorganic acid.

2. The gelatino-silver halide photographic emulsion fading preventing method of claim 1 wherein the fading preventing components consist essentially of components (1) and (2).

3. The gelatino-silver halide photographic emulsion fading preventing method of claim 1 wherein the cyanine dye is represented by the following general formula (I):



modifications can be made therein without departing from the spirit and scope thereof.

What is claimed is:

1. A method for preventing fading of a latent image in an exposed gelatino-silver halide photographic emulsion which comprises adding to said photographic emulsion (1) at least one of a monomethine or a trimethine cyanine dye having a cathode polarographic half wave potential ranging from -0.9 and -1.8 volt and an anode polarographic half wave potential lower than 1.3 volt and capable of forming J-aggregate, and (2) an organic

45 wherein  $\text{Y}_1$  and  $\text{Y}_2$  each represents an oxygen atom, a sulphur atom, a selenium atom, or a  $-\text{CH}=\text{CH}-$  group,  $\text{Z}_1$  and  $\text{Z}_2$  each represents the non-metallic atoms necessary to complete a benzene or a naphthalene nucleus,  $n$  represents an integer of 1 or 2,  $\text{X}_1^-$  represents an anionic group,  $p$  represents an integer of 1 or 2, and, when  $p$  is 1, an intramolecular salt is formed,  $\text{R}_1$  and  $\text{R}_2$  each represents a lower alkyl group, an allyl group or a substituted alkyl group, and  $\text{A}$  represents a hydrogen atom, a lower alkyl group or a substituted alkyl group; or the following general formula (II)

55



wherein  $Y_3$  represents an oxygen atom, a sulphur atom, a selenium atom,  $a = N - R_6$  group of a



group,  $R_7$  and  $R_8$  each represents a methyl group or an ethyl group,  $R_5$  and  $R_6$  each represents a lower alkyl group, an allyl group or a substituted alkyl group,  $R_3$  and  $R_4$  each represents a lower alkyl group, an allyl group or a substituted alkyl group,  $Z_3$  and  $Z_4$  each represents the non-metallic atoms necessary to complete a benzene or a naphthalene nucleus,  $X_2^-$  represents an anionic group,  $q$  represents an integer of 1 or 2, and, when  $q$  is 1 an intramolecular salt is formed,

wherein said substituted alkyl group for  $R_1, R_2, R_3, R_4, R_5$  or  $R_6$  is a hydroxyalkyl group, an acetoxyalkyl

5 substituted by a lower alkyl group having from 1 to about 6 carbon atoms, a halogen atom, an alkoxy carbonyl group, a phenyl group, or an alkoxy group having from 1 to about 4 carbon atoms, wherein said benzene or naphthalene nucleus completed by  $Z_3$  or  $Z_4$  is substituted by a hydrogen atom, a cyano group, an alkoxy carbonyl group, a trifluoromethyl group, an alkylsulfonyl group, an alkylsulfamoyl group, an alkylcarbamoyl group, an acetoxy group, a lower alkyl group, or an alk- 10 oxy group, and wherein  $X_1^-$  and  $X_2^-$  each are a bromide ion, an iodide ion, a p-toluenesulfonate ion, a perchlorate ion, an ethyl sulfate ion or a benzene sulfonate ion.

15 6. The gelatino-silver halide photographic emulsion fading preventing method of claim 4 wherein said dye of the general formula (i) or (ii) has the general formula (iii)



group, an aralkyl group, an alkyl group having a sulfo group, or an alkyl group having a carboxy group, and wherein said substituted alkyl group for

30 wherein  $Y_1, Z_1$  &  $Z_2$  are as defined in claim 2 and  $R_9$  and  $R_{10}$  each represents an alkyl group having a sulfo group; the general formula (IV)



A is an aralkyl group.

4. The gelatino-silver halide photographic emulsion fading preventing method of claim 3, wherein said organic compound is selected from the group consisting of 2,3-dihalogenomalealdehydic acids, 2,4-dichloro-S-

wherein  $R_{11}$  and  $R_{12}$  each represents a sulfoalkyl group and wherein  $W_1, W_2, W_3$  &  $W_4$  each represents a chlorine atom, a bromine atom, a trifluoromethyl group, an alkoxy carbonyl group or an alkylsulfonyl group; the general formula (V)



triazines, chloropyrimidines, chlorotriazine ring side chain containing polymers, dichlorophosphoamides,

wherein  $R_1, R_2, X_1$  and  $p$  are as defined in claim 2, or the general formula (VI)



halomethyls, phosphonitrile chlorides and 2-phenoxy-3-halogeno-malealdehydic acids.

65 wherein  $Z_1, Z_2, R_1, R_2, X_1$  and  $p$  are as defined in claim 2.

5. The gelatino-silver halide photographic emulsion fading preventing method of claim 4, wherein said benzene or naphthylene nucleus completed by  $Z_1$  or  $Z_2$  is

7. The gelatino-silver halide photographic emulsion fading preventing method of claim 4, wherein the cyanine dye is selected from the group consisting of





and



8. The gelatino-silver halide photographic emulsion fading preventing method of claim 3 wherein the organic compound is selected from the group consisting of

Cl-C-COOH

"

Cl-C-CHO



9. The gelatino-silver halide photographic emulsion fading preventing method of claim 4, wherein said cyanine dyes are present at a level ranging from  $1 \times 10^{-6}$  to  $1 \times 10^{-3}$  mol per mole of silver halide, and wherein 15 said organic compound is present at a level ranging from about 1 to about 100 g per Kg of gelatin in said emulsion on a dry basis.

10. The gelatino-silver halide photographic emulsion fading preventing method of claim 4, where said silver 20 halide is silver chlorobromide, silver bromide or silver bromoiodide.

11. The gelatino-silver halide photographic emulsion fading preventing method of claim 10, wherein said silver halide is silver bromoiodide.

25 \* \* \* \* \*